

# UNITED STATES PATENT OFFICE.

WILLIAM FREDRICK KOPER, OF CHILlicothe, OHIO.

## SOLDER-SOLVENT.

1,097,926.

Specification of Letters Patent.

Patented May 26, 1914.

No Drawing.

Application filed November 16, 1911. Serial No. 660,693.

*To all whom it may concern:*

Be it known that I, WILLIAM F. KOPER, a citizen of the United States, residing at Chillicothe, in the county of Ross and State 5 of Ohio, have invented certain new and useful Improvements in Solder-Solvents, of which the following is a specification.

My invention relates to an improvement in solvents for solder, and the object is to 10 provide a compound for removing all impurities and grit from solder, which would cause the solder to become useless for the purposes for which it is intended.

The composition of matter consists of:

|    |                  |             |
|----|------------------|-------------|
| 15 | Ammonium chlorid | 29 percent. |
|    | Sulfur           | 43 "        |
|    | Rosin            | 2 "         |
|    | Paraffin         | 9 "         |
| 20 | Mutton tallow    | 11 "        |
|    | Salt             | 5 "         |
|    | Red alkanet root | 1 "         |

which are all commingled together and made preferably into tablet form.

25 When it is desired to clean or purify a pot of metal such as solder, Babbitt metal and the like, a tablet or wafer is dropped into the metal after the metal has been heated to a molten state. The temperature of 30 the molten metal should not be excessive but to a temperature sufficient to char a piece of paper dark brown. Then after the wafer is inserted into the molten metal, the molten metal is thoroughly agitated while the wafer 35 is dissolving so as to bring all of the metal

in contact with the composition, and thereby destroy all impurities in the molten metal. The ammonium chlorid and rosin serve to prevent oxidation of the metals, and the tallow and paraffin assist in making a paste as 40 well as acting as reducing agents, while the sulfur forms a molten flux on the surface of the bath to entrain the oxidized compounds floating thereon. If solder is being used, for instance, and some impurity or foreign substance should get into the metal, when it is ready for use, it would be useless, and would have to be thrown away, but by dissolving a wafer therein containing the composition above set forth, the impurities can be removed, and thereby save the molten metal. 50

Having fully described my invention, what I claim as new and desire to secure by Letters Patent, is:—

1. A composition of matter for purifying 55 metals in a molten state, consisting of ammonium chlorid, sulfur, rosin, paraffin, mutton tallow, salt and red alkanet root.

2. A composition of matter for purifying metals in a molten state, consisting of ammonium chlorid 29%, sulfur 43%, rosin 2%, paraffin 9%, mutton tallow 11%, salt 5%, red alkanet root 1%. 60

In testimony whereof I affix my signature, in the presence of two witnesses.

WM. FREDRICK KOPER.

Witnesses:

JOHN FERDINAND BURDICK,  
GEO. P. OBERMEYER.

Copies of this patent may be obtained for five cents each, by addressing the "Commissioner of Patents, Washington, D. C."